

Oct. 21, 1941.

H. DREYFUS

2,259,518

MANUFACTURE OF ARTIFICIAL MATERIALS

Filed Oct. 10, 1936



HENRY DREYFUS  
INVENTOR

*I. Salgo & Co., Inc.*  
ATTORNEY

## UNITED STATES PATENT OFFICE

2,259,518

## MANUFACTURE OF ARTIFICIAL MATERIALS

Henry Dreyfus, London, England

Application October 10, 1936, Serial No. 105,071  
In Great Britain October 28, 1935

2 Claims.

(Cl. 18—8)

This invention relates to improvements in the manufacture of artificial materials, and particularly to improvements in processes and apparatus for the manufacture of artificial filaments, yarns and other materials by wet spinning processes.

Wet spinning processes for the manufacture of artificial filaments and other materials having a basis of organic derivatives of cellulose have been described in U. S. Patent No. 1,465,994, which employs coagulating baths containing thiocyanates, and in U. S. Patent No. 1,467,493, which describes the use of aqueous baths containing acetone, diacetone alcohol, and other solvents and latent solvents for cellulose acetate. Again, U. S. applications S. Nos. 402,785 filed October 26, 1929, and 418,414, filed January 3, 1930, and British Patents Nos. 340,326 and 340,-437, describe the use of coagulating baths or after-treatment baths containing high concentrations of solvents or non-solvent plasticisers for cellulose derivatives, while U. S. application S. No. 469,622 filed July 21, 1930, is concerned with the coagulation of artificial filaments, ribbons and other products, or their after-treatment continuously with their production by wet or dry spinning processes, in baths which contain high concentrations of solvents and salts or other substances adapted to reduce the solubility of the solvent in the non-solvent medium. U. S. application S. No. 601,043 filed March 24, 1932, describes the production of artificial filaments, threads and other products by wet spinning processes in which they are coagulated or after-treated with baths containing high concentrations of glycol monoacetate or other lower aliphatic acid esters of di- or poly-hydric alcohols, other than mono- or di-acetin, or their partial ethers.

Whereas it is common practice in the production of artificial filaments and similar products by dry-spinning processes to carry out the manufacture at a spinning speed of, for example, 300 metres per minute or more, in the production of artificial filaments and similar products by wet spinning processes, for example as described in the above specifications, it has not been practicable to obtain spinning speeds greater than about 60 up to 100 metres per minute at the most. Thus British Patent No. 340,437 describes spinning artificial filaments into an aqueous coagulating bath and passing them round a feed roller driven at a peripheral speed of 50 metres per minute, while U. S. application S. No. 469,622 filed July 21, 1930, in Example 1, refers to peripheral speeds of 25 to 50 up to 100 metres per minute.

It has now been discovered that considerably greater spinning speeds may be attained in wet spinning processes by passing the artificial fila-

ments or other materials in contact with a plurality of rollers or other forwarding devices during their travel from the shaping device to the take-up device. By this means artificial filaments may, for example, be wet spun at a speed of 150-200 metres per minute or more. The artificial filaments or other materials may contact with the forwarding devices during their travel through the coagulating bath or after emerging therefrom, for example, while they are passing through an after-treatment bath containing a softening medium or while passing through the air. In this latter case the materials are preferably sprayed with a softening medium during their travel through the air. If desired the filaments or other materials may contact with one or more forwarding devices during their passage through the coagulating medium, and with one or more forwarding devices after emerging from the coagulating medium and before reaching the take-up device. The concentration of the softening medium through which the materials pass or with which they are sprayed may change either gradually or abruptly along their path of travel. Thus filaments emerging from a coagulating bath having a high softening power, e. g. a 55-60% aqueous solution of diacetone alcohol, may be sprayed at intervals, e. g. while passing in contact with the forwarding devices, with solutions of diacetone alcohol of progressively decreasing concentration and finally with water in order to wash them. They may be taken up in a spinning box and dried in cake form or be dried by passage through a heated chamber and wound or twisted and wound on a cap spinning machine or other take-up device.

A forwarding device which has been found to yield very good results consists of a set of three rollers, the second roller of each set being positioned at a level above that of the first and third rollers so that the filaments or other products pass under the first roller, up and over the second roller, and then down and underneath the third roller. All three rollers of each set may be positioned below the surface of the coagulating or after-treatment medium, or the second roller may be above the surface, in which case the products are preferably sprayed with the medium while out of contact with the bath.

A similar forwarding device, which also yields very good results, consists of a set of three rollers, the second roller of the set being below the level of the first and third. All three rollers may be below the surface of the medium or the second only may be below, in which case the products are preferably sprayed with the medium while they are out of contact with the bath.

In general, when rollers are employed which are not immersed in a coagulating or after-treat-

ment medium it is desirable to spray them with the medium.

In addition to rendering it possible to increase considerably the rate of production of yarns and other products, e. g. foils and films, by wet spinning processes, the present invention renders it possible to effect a close control of the tension on the products during their travel from the shaping device to the bobbins or other take-up devices, and the speeds of the sets of rollers or other forwarding devices may be controlled so that e. g. the yarn or other product is stretched during the whole of its travel, or so that e. g. over portions of its travel no stretch is effected, the length of the product being maintained constant or shrinkage being allowed to take place. Moreover the invention renders it possible to reduce the tension due to friction between the liquid bath and filaments, e. g. by means of the sets of three rollers described above.

The process and apparatus of the present invention are applicable broadly to the production of artificial yarns, foils and other products by wet spinning processes, for example the processes described in the above specifications, and particularly to processes in which coagulation of the products is effected in the presence of a high concentration of a solvent or other softening agent for the base of the products, e. g. a concentration of at least 40 or 45%. Preferably an aqueous coagulating or after-treatment medium is employed. Softening agents which may be employed are acetone, methylene ethylene ether, dioxane and other volatile liquids, though preferably ethyl lactate, diacetone alcohol, glycol monoacetate, methyl glycol monoacetate and other liquids of low volatility are employed. The bath may be covered with a relatively non-volatile liquid which is immiscible with the bath, for example an oil, in order to lubricate the products and/or to prevent evaporation of softening agent or diluent, particularly when a volatile softening agent is employed, as described in U. S. application S. No. 690,122 filed September 19, 1933.

An example of a wet spinning apparatus comprising a plurality of forwarding devices according to the present invention is illustrated in the accompanying drawing, which shows a sectional elevation of a wet spinning device, an after-treatment device and a take-up device.

The apparatus comprises a vessel 1 for coagulating medium which contains a jet 2 connected through a candle filter 3 with a header or other supply of spinning solution (not shown). Towards the end of the vessel remote from the jet is provided with a set 6 of three positively driven rollers arranged at the vertices of a triangle, and above the set of rollers is arranged a spray device 5. At the end of the vessel 1 is a vessel 11 in which are mounted two sets of positively driven rollers 8 and 10, the rollers of each set being arranged at the vertices of a triangle. Above the sets of rollers are provided spray devices 7 and 9. An overflow 12 is provided in the end of the vessel 11 at such a height that the liquid level in the vessel 11 is maintained above the top of the bottom roller of each set. The apparatus also comprises a draw roller 13, a guide 14 and a spinning box 15 for taking up the yarn.

In operation the bundle of filaments 4 issuing from the jet 2 into a suitable coagulating medium, for example a 45 to 50% aqueous solution of ethyl lactate, passes round the set of roll-

ers 6 whereby they are sprayed with a suitable softening medium while passing over the middle roller of the set. From these rollers they proceed round the sets of rollers 8 and 10 where they are sprayed by means of the spray 7 and 9 and then proceed to the draw roller 13 after which they pass round the guide 14 and are taken up in the spinning box 15. The sets of rollers 6, 8 and 10 and the draw roller 13 may be rotated at such speeds that the materials are drawn down between the jet and the set of rollers 6, between each set of rollers and between the set of rollers 10 and the draw roller 13, or if desired the speeds of the rollers may be such that no stretching takes place during some portion of the travel of the materials from the jet to the draw roller. The softening medium employed for spraying may also be a 40-50% ethyl lactate solution, or media of decreasing concentration may be employed in passing from the spray 5 to the spray 9, so that a gradual decrease in the plasticity of the materials is effected. For example the materials may be sprayed at 7 with a 35-40% ethyl lactate solution and at 9 with one of 25-30%.

5 While the present invention is of particular  
importance in relation to the manufacture of  
artificial materials having a basis of cellulose  
acetate, it may also be employed in the manu-  
6 facture of artificial materials having a basis of  
cellulose formate, propionate, butyrate, nitroacetate,  
acetate-propionate, and other esters and  
mixed esters of cellulose, methyl, ethyl, butyl and  
7 benzyl celluloses and other cellulose ethers and  
mixed ethers, and ethyl cellulose acetate and  
oxyethyl cellulose acetate. Moreover, it may  
also be employed in the manufacture by wet  
8 spinning processes of artificial materials having  
a basis of other suitable substances, for example  
in the manufacture of regenerated cellulose ma-  
9 terials by the viscose process.

The term "forwarding device" is employed in the description and claims of the present application to denote a device which imparts a forward movement to the materials.

Having described my invention what I desire to secure by Letters Patent is:

1. In wet spinning apparatus for the production of artificial filaments, yarns, foils, films and similar materials, a vessel for containing coagulating liquid, a shaping device through which a spinning solution is extruded into the vessel containing the coagulating liquid, and a plurality of forwarding devices at least one of which is contained substantially within the vessel containing the coagulating liquid, each of which comprises a set of three rollers arranged at the vertices of a triangle, each of the rollers of each set being positively driven.

30 2. In wet spinning apparatus for the production of artificial filaments, yarns, foils, films and similar materials, a vessel for containing coagulating liquid, a shaping device through which a spinning solution is extruded into the vessel containing the coagulating liquid, and a plurality of forwarding devices at least one of which is contained substantially within the vessel containing the coagulating liquid, each of which comprises a set of three rollers arranged at the vertices of a triangle, each of the rollers of each set being 35 positively driven at the same speed and each of the sets of rollers being adapted to be driven at different speeds.

## HENRY DREYFUS.